

April 29, 1924.

1,492,148

N. G. WARTH

INNER TUBE

Filed Oct. 18, 1920.



*Fig. 2.*



*Fig. 3.*



*Fig. 4.*



*Fig. 5.*



*Fig. 6.*



*N. G. WARTH*  
Inventor

*By C. A. Brown & Sons*  
Attorneys

## UNITED STATES PATENT OFFICE.

NATHANIEL G. WARTH, OF COLUMBUS, OHIO.

## INNER TUBE.

Application filed October 18, 1920. Serial No. 417,677.

*To all whom it may concern:*

Be it known that I, NATHANIEL G. WARTH, a citizen of the United States, residing at Columbus, in the county of Franklin and 5 State of Ohio, have invented a new and useful Inner Tube, of which the following is a specification.

This invention relates to inner tubes for use within the casings of pneumatic tires, 10 one of the objects of the invention being to provide a light tube having combined therewith a thickness of sticky, plastic rubber compound or the like whereby the tube is rendered self healing after being punctured.

A further object is to provide a tube of this character in which the inner or exposed surface of the layer of sticky compound has a coating of vegetable or mineral fiber which 20 cooperates with said compound to provide a plugging or damming material which will flow with the compound to the perforation or puncture and aid materially in the closing thereof, and which also acts as a mat or 25 covering whereby the pressure of air within the inflated tube will result in the shifting of the compound over an extended area toward the puncture during the self healing action.

30 A further object is to provide a fibrous inner coating which serves to prevent the opposed portions of the wall of the tube from sticking together when the tube is deflated or flattened.

35 A still further object is to provide a tube having a fibrous inner layer which will operate efficiently whether the tube is a compression tube, i. e. a tube which is placed under annular compression when inflated, 40 or an expansion tube, i. e. a tube which will stretch when inflated, the said fibrous coating at no time interfering with either the compression or expansion of the tube, as would be the case should a fabric, leather, 45 or other coating of sheet material be employed.

With the foregoing and other objects in view, which will appear as the description proceeds, the invention resides in the combination and arrangement of parts and in the details of construction hereinafter described and claimed, it being understood that, within the scope of what is claimed, changes in the precise embodiment of the 50 invention shown can be made without departing from the spirit of the invention.

In the accompanying drawings the preferred form of the invention has been shown.

In said drawings—

Figure 1 is a transverse section through 60 a portion of an inner tube constituting the present invention, the adjacent part of the tire casing being also shown.

Figure 2 is a section on line 2—2, Figure 1 through a portion of the tube and casing 65 and showing the relative positions of the parts prior to inflation.

Figure 3 is a similar view showing the 70 relative positions of the parts subsequent to inflation.

Figure 4 is a similar view showing the 75 positions taken by the layers of the inner tube while being punctured.

Figure 5 is a like view showing how the parts are positioned during the withdrawal 75 of the puncturing device.

Figure 6 is a section showing the healed 80 puncture.

Referring to the figures by characters of reference 1 designates the wall of the inner 80 tube formed of cured or vulcanized rubber and applied to the inner surface of this wall is a thickness or layer of sticky plastic compound indicated at 2 and which layer can extend either partly or entirely over the 85 inner surface of the tube wall, it being essential, however, that it be arranged upon the tread and adjacent side portions of the wall. While this compound can be of any 90 of the well known viscous plastic substances either with or without rubber as an ingredient it is preferred, in the present instance, to combine with the compound a filling of granular material such as cork, comminuted 95 cured rubber or any other similar substance tending to add body to the compound. It is also intended to mix with the compound a percentage of loose vegetable or mineral fibers, the entire mixture being thoroughly impregnated with the compound so that the 100 same will be able to flow properly to a puncture in the manner hereinafter pointed out.

There is provided on the inner surface of the layer 2 an inner coating of loose fibers 105 of a mineral or vegetable nature which, when the tire is deflated, will present a soft fluffy surface so that when the tube is flattened the opposed portions of the wall thereof will not stick together. When the tube is 110 inflated, however, the pressure of the air against these loose fibers forming the inner

surface will cause them to hug close to the inner surface of the layer 2 and form a mat. As the fibers are not woven to a fabric they will not resist expansion or contraction of the compound 2 but will move therewith freely. The pressure of the air against these matted fibers will result in equal distribution of the pressure throughout the area of the compound.

10 When the tube is punctured by a nail *a*, wire or other article the point thereof while passing through the tube will force the layers of the tube inwardly from the compressed position shown in Figure 3 to the position shown in Figure 4. As the article *a* moves into the tube the sticky compound will adhere thereto and a portion of this compound will travel inwardly with the article *a*. Owing to the equal distribution of pressure through the matted fibers and against the compound, said compound will be caused to flow through a considerable area toward the entering object *a* with the result that an excessive amount of the compound will be brought to position adjacent the point of puncture. As a result of this action when the object *a* is withdrawn, as shown in Figure 5 it will drag a portion of the compound with it into the opening that has been formed in the wall 1 of the tube and some of the fibers adjacent the puncture will likewise be drawn by the compound into the opening. As the compound includes both granular and fibrous ingredients they will be ample to thoroughly plug any medium sized puncture but should the puncture be larger than ordinarily some of the fibers forming the inner coating 3 will be drawn up into the puncture and insure healing thereof. As the object *a* is withdrawn from the tire casing, indicated at *b*, said casing being of a hard non-elastic material will operate to strip from the object *a* all of the compound, etc., adhering thereto with the result that there will be left within the puncture and upon the adjacent portion of the outer surface of the wall 1 an exudation of healing material which will operate positively to prevent leakage of air. The pressure of the air within the tube and against the matted layer 3 will cause the compound to move toward the point from which the object *a* was withdrawn so that the compound will here amalgamate or flow together and, at the same time, the adjacent fibers of the inner coating *b* will work over the point of puncture and thus complete the healing operation.

60 By providing an inner coating of fibers which will form a mat when the tube is inflated, the plastic sticky compound is given the necessary support or re-enforcement to

prevent it from blowing out of the puncture. In other words the pressure of the air against the mat results in application 65 of pressure over the entire area of the plastic compound and results in the movement of this compound when under compression toward the weakest point or the point of puncture and between the fibrous mat 3 and 70 the wall 1. Without utilizing this fibrous mat the tendency of the plastic compound would not be to flow bodily toward the point of puncture. Instead the pressure of the air would tend to shift only that portion of the compound adjacent the puncture, with the result that the compound would in many cases be blown through the puncture and the sealing action would not be as reliable or efficient as in the present 80 case, and, in fact, would not take place at all should a large puncture be made in the tube. The fibers when matted as described are advantageous as compared with a fabric inner coating because they do not limit the 85 flowing action of the compound or in any way interfere with the expansion or the compression of the tube within the casing of the tire when the tube is inflated. In other words the tube will operate just as 90 efficiently in an oversized casing as in an undersized casing.

It has been found that by combining with the plastic compound a volatile substance or a substance that will dry quickly when 95 exposed to air, as for example pitch, linseed oil, albumen, gum arabic or the like, the exudation of compound produced by the sealing of the tube will become dry and thus effect a permanent seal which will enable 100 the tube to be removed from one casing, after being punctured and used in another casing and still remain air tight.

In view of the fact that animal fibers cannot stand heat during the vulcanizing 105 process it has been found desirable to use only vegetable or mineral fibers in the formation of this tube.

What is claimed is:—

A self healing inner tube for pneumatic 110 tires comprising a wall of cured rubber, a solid layer of sticky plastic compound upon the inner surface of said wall at the tread portion thereof, and an inner coating of matted loose fibers lying flat upon and 115 adhering to the inner or exposed surface of said compound.

In testimony that I claim the foregoing as my own, I have hereto affixed my signature in the presence of a witness.

NATHANIEL G. WARTH.

Witness:

HERBERT D. LAWSON.